

## UNITED STATES PATENT OFFICE

2,079,108

## TEXTILE PROCESS AND PRODUCT

Camille Dreyfus, New York, N. Y., and William Whitehead, Cumberland, Md., assignors to Celanese Corporation of America, a corporation of Delaware

No Drawing. Application April 17, 1930,  
Serial No. 445,202

## 20 Claims. (Cl. 18—54)

This invention relates to the preparation or treatment of textile materials, such as yarns or filaments made of organic derivatives of cellulose, whereby the same are rendered more amenable to textile operations or have other improved properties.

An object of our invention is to prepare or treat textile materials containing organic derivatives of cellulose so as to improve their properties.

10 A further object of our invention is to prepare or treat textile materials, particularly yarns or filaments containing cellulose acetate or other organic derivatives of cellulose by the employment of a partial higher fatty acid ester of a polyhydric alcohol, whereby the yarns or filaments are rendered more pliable and can therefore be knitted, woven or knotted more readily. Further objects of our invention will appear from the following detailed description.

20 In many processes of conversion of textile yarns, such as twisting, winding, knitting or weaving, it is desirable to apply finishes which soften and lubricate the yarns. In the case of yarns of cellulose acetate or other organic derivatives of cellulose, such finishes should preferably be hydroscopic in order to soften such yarns and should also be oleaginous in order to lubricate the same. We have found that the partial higher fatty acid esters of polyhydric alcohols, that is compounds 30 wherein not all of the hydroxyl groups of the polyhydric alcohols are substituted by the fatty acid radical, produce excellent results, when employed in finishes for such yarns, or are incorporated in the spinning solution from which they 35 are formed. Because of the presence of the unsubstituted hydroxyl group, such compounds are hydroscopic and act as softening agents for the textile material, and because they are esters of fatty acids, they have lubricating properties.

40 Moreover such compounds are miscible in all proportions with fatty acids, the glycerides of such fatty acids, and polyhydric alcohols, and therefore they can be employed in conjunction with these materials as finishes and the like.

45 In accordance with our invention, we employ partial higher fatty acid esters of polyhydric alcohols in the preparation or treatment of textile materials, particularly those containing cellulose acetate or other organic derivatives of cellulose.

50 The term partial higher fatty acid esters of polyhydric alcohols is intended to include such compounds wherein at least one of the hydroxyl groups of the polyhydric alcohols is unsubstituted. Examples of such esters are glycerine mono-

5  $C_3H_5(OH)(C_{18}H_{33}O_2)_2$ ; ethylene glycol mono-oleate, diethylene glycol mono-oleate; or other partial higher fatty acid esters such as the stearate, palmitate or ricinoleate of such polyhydric alcohols, provided that there is an unsubstituted hydroxyl group present.

In one form of our invention, the partial higher fatty acid esters of polyhydric alcohols may be added to the spinning solution or dope from which the yarns, filaments, artificial bristles or straw are 10 spun. Thus to a solution of an organic derivative of cellulose in a volatile solvent, an appropriate amount of the fatty acid ester, say from 2 to 20% of the weight of the derivative of cellulose present, may be added, and such solution be extruded 15 through orifices into an evaporative atmosphere as in dry spinning, or into a precipitating bath, as in wet spinning.

The organic derivative of cellulose employed in the textile material may be a suitable organic 20 ester of cellulose or a cellulose ether. Examples of such cellulose esters are cellulose acetate, cellulose formate, cellulose propionate and cellulose butyrate, while examples of cellulose ethers 25 are ethyl cellulose, methyl cellulose and benzyl cellulose.

As examples of solvents employed in making the spinning solution, the following are given: acetone and its mixtures with water and ethyl or methyl alcohol; chloroform and its mixtures with 30 ethyl or methyl alcohol; mixtures of ethylene dichloride and ethyl or methyl alcohol; and mixtures of dichlorethylene with ethyl or methyl alcohol. These liquids or mixtures of liquids are 35 also solvents for the higher fatty acid partial esters of polyhydric alcohols employed in this invention.

In another form of our invention, the higher fatty acid partial esters of the polyhydric alcohols 40 may be applied to the yarns, filaments or fabrics after their formation. They may be applied either alone or in admixture with other materials to the textile material. As they are strong solvents for the polyhydric alcohols themselves, fatty acids and soaps, they may be used in finishes 45 for yarns, which finishes also contain such compounds. Furthermore they may be applied to textile materials very readily from aqueous emulsions where finishing is desired of yarns, fabrics and the like. When applied as or in finishes, 50 they scour off from the textile material very readily. Since they are so readily emulsified, they may be employed with advantage in the making of printing pastes for application to fabrics in place of oils. Such polyhydric alcohol partial fatty 55

- acid esters are miscible with the polyhydric alcohols, which are solvents for fugitive dyestuffs for cellulose acetate yarns, such as the acid dyes (e. g. the sodium salt of sulfonated indigotine).
- 5 Therefore a finish may be made which contains the partial esters and the fugitive dyestuff dissolved in the polyhydric alcohol, and the same may be applied to cellulose acetate yarn for the purpose of yarn identification. Moreover the 10 partial esters of the polyhydric alcohols have sufficient solvent power for such fugitive dyestuffs so that solutions of the dyestuff in them alone may be applied to yarn both as a finish and as a fugitive tint.
- 15 Yarns, artificial straw or filaments, when prepared or treated in accordance with this invention, have great pliability as shown by the fact that such yarns may be readily knitted into a fabric containing many stitches per unit length, 20 and artificial bristles, horsehair and straw may be knotted quite tightly and bend quite severely without breaking. Moreover they do not tend to develop appreciable charges of static electricity when manipulated. Fabrics when treated or prepared in accordance with this invention have a 25 very soft handle and improved draping properties.

In order further to illustrate our invention but without being limited thereto, the following specific examples are given.

*Example I*

A finish is prepared as follows:

|                       | Parts by weight |
|-----------------------|-----------------|
| 35 Diethylene glycol  | 50              |
| Glycerine mono-oleate | 50              |

Before used both of these materials are stabilized as to the atmosphere, that is they are permitted to absorb as much moisture as they can.

40 The above mixture is applied to an acetone-soluble cellulose acetate yarn, by causing such yarn to pass over wicks, rollers or other suitable devices for applying such mixture, in their transit to a winding machine. The amount of 45 finish applied is 10% of the weight of the yarn. The yarn so treated is more pliable, knits with less distortion and irregularities, takes high twists more smoothly and generally exhibits improved properties from a textile manipulation 50 point of view. Fabrics en greige comprising this yarn scour oil-free very readily and also wet out rapidly.

If instead of employing the above mixture, glycerine mono-oleate alone is applied in amounts of about 10% of the weight of the yarn, similar 55 benefits are obtained.

*Example II*

60 The process of Example I is repeated, with the exception that the finish also contains 2 parts by weight of soaps such as the oleate of sodium, potassium or triethanolamine. Similar improved results are obtained. The fabrics, yarns and the like so treated scour and wet out with remarkable ease, the finish diffusing from the yarn 65 quite readily, even in cold water.

*Example III*

70 The following spinning solution is prepared

|                          | Parts by weight |
|--------------------------|-----------------|
| Cellulose acetate        | 25              |
| Acetone                  | 72              |
| Water                    | 3               |
| 75 Glycerine mono-oleate | 1.25            |

The solution is thoroughly mixed and filtered and then is forced through orifices of a spinneret into a warm evaporative atmosphere where the acetone and water are substantially evaporated off. The filaments thus formed are twisted to form 5 yarn. The yarn so formed is immediately ready for textile operations and has the improved properties of the yarn described in the preceding examples. The yarn also has the property of delustering or assuming a subdued lustre, when 10 scoured or dyed in aqueous baths at temperatures below boiling, such as at 75° C. or over, which property is not shared by yarns prepared from spinning solutions not containing the glycerine mono-oleate.

15 It is to be understood that the foregoing examples are given merely by way of illustration and that many variations may be made therein without departing from the spirit of our invention.

20 Having described our invention, what we desire to secure by Letters Patent is:

1. The process of improving the properties of 25 artificial materials containing organic derivatives of cellulose, comprising incorporating a partial higher fatty acid ester of a polyhydric alcohol in said artificial materials containing organic derivatives of cellulose.

2. The process of improving the properties of 30 artificial materials containing cellulose acetate, comprising incorporating a partial higher fatty acid ester of a polyhydric alcohol in said artificial material containing cellulose acetate.

3. The process of improving the properties of 35 artificial materials containing cellulose acetate, comprising incorporating a partial higher fatty acid ester of glycerine in said artificial materials containing cellulose acetate.

4. The process of improving the properties of 40 artificial materials containing cellulose acetate, comprising incorporating glycerine mono-oleate in said artificial materials containing cellulose acetate.

5. The process of improving the properties of 45 textile materials comprising incorporating a partial higher fatty acid ester of a polyhydric alcohol in said textile materials.

6. The process of improving the properties of 50 textile materials containing organic derivatives of cellulose, comprising incorporating a partial higher fatty acid ester of a polyhydric alcohol in textile material containing organic derivatives of cellulose.

7. The process of improving the properties of 55 textile materials containing cellulose acetate, comprising incorporating a partial higher fatty acid ester of a polyhydric alcohol in said textile material containing cellulose acetate.

8. The process of improving the properties of 60 textile materials containing cellulose acetate, comprising incorporating a partial higher fatty acid ester of glycerine in said textile material containing cellulose acetate.

9. The process of improving the properties of 65 textile materials containing cellulose acetate, comprising incorporating glycerine mono-oleate in said textile materials containing cellulose acetate.

10. Process of forming artificial materials comprising shaping a solution containing an organic derivative of cellulose and a partial higher fatty acid ester of a polyhydric alcohol and setting the same into solid form.

11. Process of forming artificial materials comprising shaping a solution containing cellulose 75

- acetate and a partial higher fatty acid ester of a polyhydric alcohol and setting the same into solid form.
12. Process of forming artificial filaments comprising extruding a solution containing cellulose acetate and glycerine mono-oleate into a setting medium.
13. Process of forming a textile material of reduced lustre comprising subjecting organic derivative of cellulose textile material containing a partial higher fatty acid ester of a polyhydric alcohol to the action of an aqueous fluid at elevated temperatures.
14. Process of forming a textile material of reduced lustre comprising subjecting cellulose acetate textile material containing a partial higher fatty acid ester of a polyhydric alcohol to the action of an aqueous fluid at elevated temperatures.
15. Textile materials containing a partial higher fatty acid ester of a polyhydric alcohol.
16. Artificial materials containing organic derivatives of cellulose and a partial higher fatty acid ester of a polyhydric alcohol.
17. Artificial materials containing cellulose acetate and a partial higher fatty acid ester of a polyhydric alcohol.
18. Yarns or filaments containing cellulose acetate of increased pliability and containing a partial higher fatty acid ester of a polyhydric alcohol.
19. Yarns or filaments containing cellulose acetate of increased pliability and containing glycerine mono-oleate.
20. Textile materials containing glycerol mono-oleate.

CAMILLE DREYFUS.  
WILLIAM WHITEHEAD.